

## UNITED STATES PATENT OFFICE

2,279,604

## PROCESS FOR PRODUCING COPYING PAPER

Rudolf Wälti, Basel, Switzerland

No Drawing. Application September 7, 1937, Serial No. 162,764. In Germany September 16, 1936

## 1 Claim. (Cl. 91—68)

The object of my invention is the production of a liquid copying composition to be applied in the form of a thin and smudge-proof coat to the surfaces of writing or drawing papers, in particular typewriting papers, as an improved substitute for the commonly used carbon paper.

I have found that I was able to eliminate the various inadequacies and disadvantages inherent in and connected with the manufacture and use of the common carbon paper by substituting for the waxy-oily or fatty dye-paste coating of the latter aqueous solutions or emulsions of substances forming elastic films, such as, e. g., liquid latex. Since I apply or spread on the dye-carrying paste in the cold state and since the latter, aside from the film-producing component and the dye, contains only water, the ordinary apparatus used for dyeing the paper also may be employed for the purpose of applying this dye-carrying paste. Such a latter coat, applied in combination with such substances as, e. g., latex, does not penetrate through the body of the sheet, is perfectly smudge-proof and, when using and employing relatively cheap dyes such as, e. g., carbon black, extremely cheap to manufacture. Thanks to these latter properties the dye-carrying film, which heretofore has been applied to the one side of the ordinary carbon paper for the purpose of copying letters, figures and drawings onto a second sheet, may be applied now directly onto the back of the original writing sheet. The latter, therefore, is taking the place of the carbon paper heretofore inserted between the writing and the copying sheets.

A process has been known for some time, viz. the so-called "Transcrit"-process, which also operates without the use of carbon paper. This process, mostly used only for the local printing on of the copying dye-coat, is employing, however, the very same and relatively expensive dye-film of the carbon paper, i. e. a dye containing waxes, oils or fats as binding agents. For applying such a latter coat, furthermore, a set of special and relatively complicated machines is required which are eliminated in the process according to the present invention.

A further pronounced difference between the present and the known processes is that the paper of the former has to be coated on both sides. The dye on the back of the sheet, bound by the film-producing substance such as, e. g., latex, does not copy onto ordinary copying paper; which, by the way, also is the effect of its smudge-proofness, since the said dye cannot be readily rubbed off. In order to obtain a copy,

one therefore also has to apply a thin coat of a film-producing substance to the surface of the sheet to be copied on.

It yet may be mentioned that by means of the writing and copying paper treated with the solution or emulsion according to my present invention there may be made just as many copies as by means of the ordinary carbon paper used heretofore.

Paper treated in accordance with the present invention, such as, e. g., coated with a solution of latex, may be written and printed on like any ordinary paper treated with glue. The process, therefore, also may be made use of in making forms to be copied either by hand or by means of the typewriter.

The process is, e. g., applied as follows: The one side of a roll or sheet of paper first is impregnated with a solution containing, per litre, 20 grams of Revertex T (a latex-concentrate containing about 75% dry substance) to which, if need be and so desired, protective agents against aging, e. g. phenyl-betanaphthylamin, are added. After impregnating the sheet is dried, and the dye-paste is applied to the back of the sheet. The impregnating of the front and rear side also may be accomplished by means of special machines in one operation, for example by a simultaneous spraying on of the dye-dispensing and 20 the dye-receiving film coat. It also is possible to apply the one or the other of the latter coats only in certain places instead of over the entire surface of the paper. For this latter operation one suitably adds a thickening agent to the latex-solutions such as, e. g., glue. Dyes preferably to be used are: carbon black, mineral colors appearing on the market under the name of Ultramarine, Hansa-colors, Vulkan-colors and the like which are free from manganese and copper and 30 which do not precipitate the caoutchouc. Adding a dispersing agent (sulfonation-products of fats and condensed aromatic solvents, fat-alcohol sulfonates etc. known to the trade under the names Melioran, Igepon T, Peregol O and so on) has proven of excellent value for finely distributing the dyes in the aqueous solution.

In preparing the dye-paste composition I prefer, by way of example, to use the ingredients in about the following proportions and to add them in the following manner—viz., 60 grams of carbon black, 100 cc. of water and 40 grams of a 10% Igepon T solution are made into a paste and, by stirring, added to a solution of 40 grams Revertex T in 760 cc. of water. The quantity obtained then is 1 kilogram. To this dye-paste also, in

any given case, a protective means against aging may be added.

The quantities of carbon black and Revertex T given in the above example obviously may be increased or decreased according to requirements. One also may proceed by first coating the paper with the dye-paste and then applying the 2% Revertex T solution.

A variation of the process described consists in using unglued paper, substituting the passing of the paper through a Revertex-solution for the gluing operation. After such a passage the coat is dried and then the dye-film spread on.

An example for the Revertex-solution used is as follows: To 60 grams of Revertex 940 cc. of water are slowly added, the quantity obtained is 1 kilogram.

An example for dye-paste is as follows: 60 grams of carbon black, 100 cc. of water and 40 grams of a 10% Igepon T solution are made into a paste which is added, by stirring, to a solution of 30 grams Revertex T in 770 cc. of water. The quantity obtained is 1 kilogram.

In the following claim the term "dispersion" means either a solution or an emulsion.

What I claim and desire to secure by Letters Patent is:

A process for producing copying paper comprising coating one side of said paper with an aqueous dispersion of latex and then coating the other side of said paper with an aqueous dispersion of latex and a coloring substance free from a precipitating action upon said latex.

RUDOLF WÄLTI.